

## UNITED STATES PATENT OFFICE

2,243,213

PROCESS OF PRODUCING FAST DYEINGS ON  
CELLULOSE ESTERS AND ETHERS AND  
THE DYED FIBER OBTAINED THEREBY

Georg Kränzlein and Carl Josef Müller, Frankfurt-on-the-Main, and Werner Kirst, Königstein in Taunus, Germany, assignors to General Aniline & Film Corporation, New York, N. Y., a corporation of Delaware

No Drawing. Application November 9, 1939, Serial No. 303,538. In Germany December 1, 1938

10 Claims. (Cl. 8—48)

The present invention relates to a process of producing fast dyeings on cellulose esters and ethers and to the dyed fiber obtained thereby.

As is known, fast dyeing may be produced on cellulose esters and ethers by applying to this material an aromatic compound containing an amino-group capable of being diazotized, then diazotizing the compound on the fiber and developing it to the azo-dyestuff by treatment with a coupling component, as for instance, 2,3-hydroxynaphthoic acid or beta-naphthol.

This invention relates to the production of fast dyeings on cellulose esters or ethers in a much simpler manner by applying to the cellulose ester or ether or dissolving therein an azo-dyestuff which does not contain a sulfonic acid group, but contains in the molecule an amino-group capable of being diazotized and a free position capable of coupling with diazo-compounds, then diazotizing the compound and causing the diazo-compound obtained to combine with itself, if desired by adding to the diazo-bath an agent neutralizing the acid or having an alkaline action, after the diazotization is finished, or by passing the diazotized goods through a bath containing one of the said agents.

The azo-dyestuff may be applied to the fiber in an acid or neutral solution or suspension. The diazotization is performed by means of the usual agents. The azo-dyestuffs may also be added to the spinning solution.

In comparison with the known process the new process is distinguished by its simple mode of application, since the after-treatment with a developer and, accordingly, a coupling bath with a separate coupling component can be dispensed with. Moreover, the fastness to wet-processing

of the dyeings obtained by this invention is superior to that of the known dyeings obtainable by using a separate heterogeneous coupling component.

5 The following example serves to illustrate the invention, but it is not intended to limit it thereto:

1 kilo of acetate silk yarn is treated for one hour at about 80° C. with a suspension containing in 25 liters of water 50 grams of a finely dispersed azo-dyestuff having the following constitution:



20 (obtainable by coupling diazotized 1-amino-2-methoxy-4-nitrobenzene in an acid medium with 2-amino-5-hydroxynaphthalene and subsequently reducing the nitro-group). The yarn is then rinsed and introduced into a bath containing in 30 liters of cold water 30 grams of sodium nitrite and 80 cc. of concentrated hydrochloric acid. After one hour the diazotization is complete.

25 The material is then centrifuged and the dyeing is developed in a cold bath containing in 30 liters of water 80 cc. of ammonia of 25 per cent strength. The goods are then centrifuged and dried. A black-brown dyeing of good properties of fastness, especially of very good fastness to wet-processing is obtained.

30 35 The following table indicates a number of other dyeings obtainable by this invention:

|    | Parent component                                                       | Shade                                                                     |
|----|------------------------------------------------------------------------|---------------------------------------------------------------------------|
| 1  | 1-amino-4-nitrobenzene acid<br>or<br>1-amino-4-acetylaminobenzene acid | 2-amino-5-hydroxynaphthalene, reduced, Brown-black.                       |
| 2  | 1-amino-2-chloro-4-nitrobenzene acid                                   | 2-amino-5-hydroxynaphthalene, saponified. Black-brown.                    |
| 3  | 1,4-diamino-3,5-dichlorobenzene acid                                   | 2-amino-5-hydroxynaphthalene. Violet-brown.                               |
| 4  | 1-amino-3-nitro-6-methylbenzene acid                                   | 2-amino-5-hydroxynaphthalene, reduced. Brown.                             |
| 5  | 1-amino-4-nitro-6-methylbenzene acid                                   | 2-amino-5-hydroxynaphthalene, reduced. Violet-brown.                      |
| 6  | 4'-nitro-4-aminodiphenylamine acid                                     | 2-amino-5-hydroxynaphthalene, reduced. Black.                             |
| 7  | 1-amino-4-nitro-2-methoxy-5-chlorobenzene                              | 2-amino-5-hydroxynaphthalene, reduced. Violet-black.                      |
| 8  | 2-amino-5-hydroxynaphthalene                                           | n-amino-acetanilide. Brown.                                               |
| 9  | 2-amino-5-hydroxynaphthalene                                           | 1-aminonaphthalene. Violet-brown.                                         |
| 10 | 2-amino-5-hydroxynaphthalene                                           | aniline, according to the statements in German Patent No. 131,860. Brown. |
| 11 | 2-amino-5-hydroxynaphthalene                                           | 1-amino-3,5-dimethylbenzene. Do.                                          |
| 12 | 2-amino-5-hydroxynaphthalene                                           | 1-amino-2-methoxy-5-methylbenzene. Do.                                    |
| 13 | 2-amino-8-hydroxynaphthalene                                           | 1-amino-2-methoxy-5-methylbenzene. Do.                                    |

|    | Parent component                                                                                                                          | Shade            |
|----|-------------------------------------------------------------------------------------------------------------------------------------------|------------------|
| 14 | alkaline<br>2-amino-8-acetoxy-naphthalene → 2-amino-8-hydroxynaphthalene, saponified.                                                     | Violet-black.    |
| 15 | 1-amino-8-hydroxynaphthalene → aniline, according to the statements in German Patent No. 131,860.                                         | Brown.           |
| 16 | 2-amino-8-hydroxynaphthalene → 1-amino-naphthalene.                                                                                       | Black-brown.     |
| 17 | 2-amino-8-hydroxynaphthalene → 1-amino-3,5-dimethylbenzene.                                                                               | Brown.           |
| 18 | 2-amino-8-hydroxynaphthalene → 3-amino-acetanilide.                                                                                       | Reddish-brown.   |
| 19 | 2-amino-8-hydroxynaphthalene → 1-amino-2,5-dimethoxybenzene.                                                                              | Do.              |
| 20 | 1-amino-5-hydroxynaphthalene → 1-amino-2-methoxy-5-methylbenzene.                                                                         | Red-brown.       |
| 21 | 1-(3'-aminophenyl)-3-methyl-5-pyrazolone → 1-aminonaphthalene acid                                                                        | Brown.           |
| 22 | 1-amino-4-nitro-2-methoxybenzene → 2-amino-7-hydroxynaphthalene, reduced.                                                                 | Brown-black.     |
| 23 | 1-amino-4-nitro-2-chlorobenzene → 1,3-dihydroxybenzene, reduced.                                                                          | Brown.           |
| 24 | 1-amino-4-nitro-2-methoxybenzene → phenol, reduced.                                                                                       | Do.              |
| 25 | 4-aminobenzoylacetylaminobenzene → 1-amino-3-methoxybenzene.                                                                              | Brown-orange.    |
| 26 | Sulfurous acid ester of 1-amino-8-hydroxynaphthalene → 2-amino-4-methoxy-1-methylbenzene, saponified.                                     | Brown.           |
| 27 | Aniline → 1-amino-5-hydroxynaphthalene acid                                                                                               | Red-brown.       |
| 28 | Aniline → 2-amino-5-hydroxynaphthalene acid                                                                                               | Yellow-brown.    |
| 29 | Aniline → 1-amino-7-hydroxynaphthalene acid                                                                                               | Brown.           |
| 30 | Aniline → 2-amino-7-hydroxynaphthalene acid                                                                                               | Yellow-brown.    |
| 31 | 1-amino-4-acetylaminobenzene → 2-amino-5-hydroxynaphthalene acid                                                                          | Brown-orange.    |
| 32 | 1-amino-3-acetylaminobenzene → 2-amino-5-hydroxynaphthalene acid                                                                          | Orange-brown.    |
| 33 | 1-amino-3-acetylaminobenzene → 2-amino-5-hydroxynaphthalene, saponified.                                                                  | Red-brown.       |
| 34 | 4-aminophenol → 2-amino-4-methoxy-1-methylbenzene.                                                                                        | Copper-brown.    |
| 35 | 3-aminophenol → 1-naphthylamine.                                                                                                          | Brown.           |
| 36 | 4-aminophenol → 1-naphthylamine.                                                                                                          | Olive-brown.     |
| 37 | 4-nitroaniline → phenol, reduced.                                                                                                         | Yellow-brown.    |
| 38 | 3-nitroaniline → phenol, reduced.                                                                                                         | Brownish-yellow. |
| 39 | 4-nitroaniline → 1,5-naphthylenediamine.                                                                                                  | Brown.           |
| 40 | 2-nitro-4-methoxy-1-aminobenzene → 1,5-naphthylenediamine.                                                                                | Do.              |
| 41 | 2-nitro-4-methoxy-1-aminobenzene → 1,5-naphthylenediamine, reduced.                                                                       | Do.              |
| 42 | 3-nitroaniline → 1-amino-7-hydroxynaphthalene, reduced,<br>or<br>1-amino-3-acetylaminobenzene → 1-amino-7-hydroxynaphthalene, saponified. | Do.              |
| 43 | 4-nitroaniline → 1-amino-7-hydroxynaphthalene, reduced,<br>or<br>1-amino-4-acetylaminobenzene → 1-amino-7-hydroxynaphthalene, saponified. | Red-brown.       |
| 44 | 1-amino-2-methoxy-4-nitrobenzene → 1-amino-7-hydroxynaphthalene, reduced.                                                                 | Do.              |
| 45 | 2-amino-5-hydroxynaphthalene → 1-amino-2-methoxy-5-methoxybenzene.                                                                        | Brown.           |
| 46 | 2-amino-5-hydroxynaphthalene → 1-amino-2-methoxy-5-methoxybenzene.                                                                        | Violet-brown.    |
| 47 | 1-amino-4-nitro-2-chlorobenzene → 2-amino-5-hydroxynaphthalene.                                                                           | Brown-orange.    |
| 48 | 3-nitroaniline → 1,3-dihydroxybenzene, reduced.                                                                                           | Brown-red.       |
| 49 | 4-nitroaniline → 1,3-dihydroxybenzene, reduced.                                                                                           | Violet-brown.    |
| 50 | 4'-nitro-2,5-dimethoxy-4-aminoazobenzene → 1,3-dihydroxybenzene, reduced.                                                                 | Red-brown.       |
| 51 | aniline → 1,3-diaminobenzene.                                                                                                             | Brown.           |
| 52 | 3-nitroaniline → 1,3-diaminobenzene, reduced,<br>or<br>1-amino-3-acetylaminobenzene → 1,3-diaminobenzene, saponified.                     | Red-brown.       |
| 53 | 3-nitroaniline → 2-methyl-5-methoxy-1-aminobenzene.                                                                                       | Brown.           |
| 54 | 3-nitroaniline → 2,4-dimethyl-1-aminobenzene.                                                                                             | Yellow-brown.    |
| 55 | Bismarck brown.                                                                                                                           | Do.              |
| 56 | 2-nitro-4-amino-1-methylbenzene → 1,5-naphthylenediamine.                                                                                 | Brown.           |
| 57 | 3-aminophenol → 1-(3'-aminophenyl)-3-methyl-5-pyrazolone.                                                                                 | Orange.          |

We claim:

1. The process which comprises applying to 50 fibrous material of the group consisting of cellulose esters and ethers a mono-azo-dyestuff which does not contain a sulfonic acid group, but contains in the molecule an amino-group capable of being diazotized and a free position capable of coupling with diazo-compounds, then diazotizing the compound on the fiber and causing the diazo-compound obtained to combine with itself by an alkaline treatment.

2. The process which comprises applying to 60 fibrous material of the group consisting of cellulose esters and ethers a mono-azo-dyestuff which does not contain a sulfonic acid group, but contains in the molecule an amino-group capable of being diazotized and a free position capable of coupling with diazo-compounds, then diazotizing the compound on the fiber and causing the diazo-compound obtained to combine with itself by passing the diazotized goods through a bath having an alkaline action subsequently to the 70 diazotization process.

3. The process which comprises applying to cellulose esters the azo-dyestuff obtainable by coupling diazotized 3-aminophenol with 1-(3'-aminophenyl)-3-methyl-5-pyrazolone, then 75

diazotizing the azo-dyestuff on the fiber and causing the diazo-compound obtained to combine with itself by an alkaline treatment.

4. The process which comprises applying to cellulose esters the azo-dyestuff obtainable by coupling diazotized 1-amino-4-acetylaminobenzene in an acid medium with 1-amino-7-hydroxynaphthalene and subsequently splitting off the acetyl-group by saponification, then diazotizing the azo-dyestuff on the fiber and causing the diazo-compound obtained to combine with itself by an alkaline treatment.

5. The process which comprises applying to cellulose esters the azo-dyestuff obtainable by coupling diazotized 3-amino-phenol with 1-naphthylamine, then diazotizing the azo-dyestuff on the fiber and causing the diazo-compound obtained to combine with itself by an alkaline treatment.

6. Fibrous material of the group consisting of cellulose esters and ethers dyed with an azo-dyestuff obtainable on the fiber by the process claimed in claim 1.

7. Fibrous material of the group consisting of cellulose esters and ethers dyed with an azo-dyestuff obtainable on the fiber by the process claimed in claim 2.

8. Cellulose esters dyed with an azo-dyestuff obtainable on the fiber by the process claimed in claim 3.

9. Cellulose esters dyed with an azo-dyestuff obtainable on the fiber by the process claimed in claim 4.

10. Cellulose esters dyed with an azo-dyestuff obtainable on the fiber by the process claimed in claim 5.

GEORG KRÄNZLEIN.  
CARL JOSEF MÜLLER.  
WERNER KIRST.